

Patented Apr. 15, 1924.

1,490,362

# UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MAINE.

## WATERPROOF FIBERBOARD.

No Drawing.

Application filed December 8, 1922. Serial No. 605,721.

To all whom it may concern:

Be it known that I, ALBERT L. CLAPP, a citizen of the United States, residing at Danvers, in the county of Essex and State of Massachusetts, have invented new and useful Improvements in Waterproof Fiberboard, of which the following is a specification.

This invention has for its object the utilization of material for which there has been no commercial use, namely, box toe waste, i. e., the scraps left after cutting box-toe blanks from a sheet of fibrous material containing bitumens, resins, waxes, or other thermo-plastic stiffening agents, alone or in admixture. It has hitherto been the practice, in the manufacture of box-toes, to form a sheet of fibrous material, such as felt formed either on a felting machine or a paper machine, to impregnate or saturate the sheet with a thermo-plastic compound, adapted to be softened upon the application of moderate heat, and then to cut the box-toe blanks of appropriate size and shape from the sheet, and in some cases to subject such blanks to a calendering operation. Due to the shape of the blanks, there is necessarily a wastage of the sheet material due to the formation of scraps and cuttings, for which no use has heretofore been found. Attempt has been made by the use of a solvent to extract the valuable gums, resins or other stiffening agents from the waste scrap material, but this has proved commercially to possess little value, due to the inflammability of the solvent, the cost of recovery, and the other necessary operations which are expensive. Then, again, the stiffening agent usually comprises several ingredients blended together to impart to the box toe the desired characteristics, and these ingredients may be varied according to the varying costs thereof. Among these thermo-plastic materials are montan and carnauba wax, common or blown asphalt, rosin and copal-resin, resin soaps, drying oils, etc., some or all of which, included by the term thermo-plastic compound, are used in varying proportions, to produce a compound or mixture which will readily penetrate the fibrous sheet, soften at a moderate temperature, while not affected by body or solar heat, set rapidly when cold, and impart stiffness and rigidity to the molded toe box. Such compounds are usually characterized

by a relatively short melting point lag, though they have no sharp or critical melting and solidifying points.

I have found that it is possible to use such waste box-toe material in the production of a water-repellent fiberboard for a number of uses in the arts, wherein both the fibrous material and the thermo-plastic compound possess great value. Ordinarily the proportion of thermo-plastic compound to fiber by weight is relatively large, and although additional fibrous material is supplied for the manufacture of fiberboard, the thermo-plastic compound is sufficient, when coalesced, in the sheet, to furnish the necessary qualities.

After much experimentation, I have found that it is possible to disintegrate the box-toe waste by grinding it while dry in a suitable grinding machine, such as an Abbe grinder. It is desirable from time to time to throw a handful of talc into the grinder to prevent the thermo-plastic compound from sticking to the knives. When disintegrated to a relatively fine dry state, the material is now ready for use.

I place in a beating engine a quantity of cellulose fiber, such, for example, as chemical wood pulp, or sulphite, or sulphate screenings, waste kraft or manilla paper, or other paper making stock, together with sufficient water to insure its circulation, and preferably subject the stock to a prolonged beating sufficient to produce a fairly hydrated or slow stock. Then while continuing the beating operation, I add (say four parts) a quantity of the disintegrated box-toe waste, and thoroughly mix it with the hydrated paper stock until a homogeneous pulpy mass is produced. The stock is now sheeted by any approved paper machine, such as a wet machine, a multi-cylinder machine, or a Fourdrinier machine. When first formed and dried, it is relatively porous, but I now subject the sheet to both heat and pressure, as by the use of heated rolls, by which the thermo-plastic compound, which is distributed throughout the fibers of the sheet, is fluxed or softened and coalesced into a state of continuity throughout the sheet, so as to enclose the fibers and protect them against the access of moisture. In the foregoing example, the mucilaginous hydrate on the cellulose fibers and fibrillæ is sufficient to retain

85

90

95

100

105

110

in the pulp those particles of the thermoplastic compound which were freed from adherence to the fibers by the grinding operation, during the forming of the sheet and 5 the removal of water therefrom, but the extent to which the hydration of the cellulosic material is carried on, depends to some extent upon the proportion of the cellulosic material to the box-toe waste. These proportions may vary considerably from 20 to 10 40 parts cellulosic stock, and 80 to 60 parts box-toe waste, by dry weight.

In many cases I regard it as desirable to 15 use some additional device for fixing the thermo-plastic particles on the fibers to prevent their waste with the white water, since I may also thereby reduce the length of the beating and decrease the extent of colloidal hydration. To this end, I add to the stock 20 in the beater and incorporate therein a suitable sizing compound, which I then precipitate by a suitable precipitating agent, so that the free particles of thermo-plastic compound are coagulated, carried down and 25 fixed upon the fibers. I employ a rosin size, or silicate of soda, or both, as the sizing compound, and precipitate the same with alum or other suitable precipitant.

As indicating the proportions which may 30 be used, the following will serve as examples, though it will be understood that these proportions may be greatly increased.

*Example I.*

35 80 parts box-toe waste  
20 parts sulphate pulp  
2 parts silicate of soda  
10 parts sodium resinate (rosin size)  
15 parts alum  
40 and such coloring matter in the form of  
pigments or dyes as may be desired.

*Example II.*

45 70 parts box-toe waste  
30 parts sulphite pulp  
10 parts rosin size  
2 parts silicate of soda  
15 parts alum  
50 and pigments or dyes.

*Example III.*

20-40 parts sulphite pulp, beaten from 2  
to 4 hours  
80-60 parts box-toe waste.  
55 The final product forms, after subjection  
to heat and pressure, a hard dense highly  
water-repellent or water-proof fiberboard,  
which may be molded, and which may be

used in the manufacture of trunks, containers, automobile flooring, etc., and which 60 lends itself to many other uses in the arts.

What I claim is:

1. A process of making fiberboard which comprises disintegrating box-toe waste having a thermo-plastic compound incorporated 65 therein, forming an aqueous pulp of said disintegrated material together with cellulosic material, and sheeting said pulp on a paper machine.

2. A process of making fiberboard which 70 comprises disintegrating box-toe waste having a thermo-plastic compound incorporated therein, while maintaining said waste in a dry state, pulping said disintegrated material together with cellulosic material and 75 water, and forming said pulp into a sheet.

3. A process of making fiberboard which comprises disintegrating box-toe waste having a thermo-plastic compound incorporated 80 therein, while maintaining said waste in a dry state, pulping said disintegrated material together with cellulosic material and water, forming said pulp into a sheet, and subjecting such sheet to heat and pressure to 85 flux and cause the coalescence of the thermo-plastic compound.

4. A process of making fiberboard which comprises disintegrating box-toe waste having a thermo-plastic compound incorporated 90 therein, beating cellulosic material with water to form a pulp, incorporating the disintegrated waste material together with a sizing compound in said pulp, adding a precipitating agent, and then sheeting the resultant 95 pulpy mass on a paper machine.

5. A process of making fiberboard which comprises disintegrating box-toe waste having a thermo-plastic compound incorporated therein, beating cellulosic material with water to form a pulp, incorporating the disintegrated waste material together with a sizing compound in said pulp, adding a precipitating agent, sheeting the resultant 100 pulpy mass on a paper machine, and finally 105 by heat and pressure fluxing the particles of thermo-plastic compound incorporated in the sheet.

6. A water-repellant fiberboard comprising cellulosic material, and disintegrated fibrous box-toe waste having a thermo-plastic compound incorporated therein, all with the fibers in felted relation and protected by the said thermo-plastic compound.

In testimony whereof I have affixed my signature.

ALBERT L. CLAPP.